# EUROPEAN PATENT SPECIFICATION

(11) **EP 1 702 101 B1**
(45) Date of publication and mention of the grant of the patent: **25.02.2009**
(21) Application number: 04805227.8
(22) Date of filing: 22.12.2004
(51) Int. Cl.: D21C 1/06, D21C 3/02, D21C 3/22

(54) **BATCH PROCESS FOR PREPARING PULP**
DISKONTINUIERLICHES VERFAHREN ZUR HERSTELLUNG VON ZELLSTOFF
PROCEDE DISCONTINU DE PREPARATION DE PATE

(30) Priority: 31.12.2003 FI 20031929
(43) Date of publication of application: 20.09.2006
(73) Proprietor: GLV Finance Hungary Kft., Luxembourg Branch, 5365 Munsbach (LU)
(72) Inventor: MARTIKAINEN, Seppo, 98440 Kallaanvaara (FI); TIKKA, Panu, FI-02160 ESPOO (FI); TIMONEN, Olli, FI-26100 RAUMA (FI); SVEDMAN, Mikael, FI-65100 VASA (FI)
(74) Representative: Hano, Christian
(86) International application number: PCT/FI2004/050196
(87) International publication number: WO 2005/064075

(56) References cited:
- EP-A1- 0 520 452
- EP-A1- 0 810 321
- WO-A1-01/25531
- WO-A1-99/14423
- US-A- 4 578 149
- US-B1- 6 350 348

## Description

### FIELD OF THE INVENTION

The present invention relates to a process for preparing kraft pulp in which lignocellulosic material is treated with recycled process liquors, polysulfide and fresh re-causticized white liquor for removing lignin therefrom. More particularly, the present invention relates to the use of polysulfide white liquor (or another polysulfide source) in the early stages of modern displacement kraft batch cooking, and the advantage thereof in terms of improved pulp yield.

### BACKGROUND OF THE INVENTION

In the various kraft pulping processes, lignocellulosic material, most commonly wood chips, is generally treated at elevated temperatures with alkaline cooking liquor containing sodium hydroxide and sodium hydrogen sulfide, called white liquor. In these processes a significant part of the cellulosic material, especially hemicelluloses, are partly lost due to reactions with the white liquor. In kraft pulping conditions hemicelluloses undergo alkaline peeling reactions, de-polymerization, in which the hemicelluloses are dissolved as organic acids into the cooking liquor. A known fact is that by a polysulfide treatment, hemicelluloses are stabilized and are thereafter more resistant to cooking liquor in kraft cooking conditions, which leads to higher yield from the processes lignocellulosic substance input.

In graft pulping processes, fresh cooking liquor is obtained from the recovery furnace's inorganic smelt, which is dissolved in water and causticized to produce white liquor. Polysulfide-containing white liquor is obtained from causticized white liquor by various processes, which partially oxidize the liquor's sodium sulfide into polysulfide. These processes typically use oxidation catalysts to polymerize the white liquor's hydrogen sulfide.. Also, polysulfide can be produced directly by elemental sulfur addition into white liquor. Polysulfide-containing white liquor is called polysulfide white liquor or orange liquor.

The use of polysulfide white liquor has been quite straightforward in conventional kraft cooking operations. The normal white liquor has been converted to polysulfide white liquor, and that liquor has been used in the same manner as normal white liquor. After the impregnation into the wood chips in the digester and during the temperature rise to above 100 °C, the polysulfide has reacted with the carbohydrates making them less vulnerable to alkaline degradation. Later during the cook, when temperature has risen over 140 °C, the rest of the polysulfide has rapidly broken down through thermal decomposition. As all the conventional cooking systems have used cooking liquors having initial temperatures well below 100 °C and the temperature in the digester has been elevated slowly or in steps, the polysulfide has had the possibility to react and facilitate higher pulp yield.

However, the development of the batch cooking systems has caused a major deviation from the conventional cooking technology: White liquor is introduced into the digester as "hot white liquor", which has been heated up using the heat ofthe previously generated spent liquor, and steam. For the purpose of this disclosure, "hot" is meant to designate a liquor having a temperature above its boiling point at ambient pressure, i.e. a liquor that must be stored in a pressurized vessel.

The hot white liquor temperature in typical displacement batch cooking is 140-180 °C. From the displacement batch process point of view, polysulfide has been an impossible chemical. Polysulfide is unstable at higher temperatures, for instance at those used in kraft cooking; the chemical begins to break down at temperatures above 100°C, and it degrades completely in a few minutes at 150 °C. Thus at the typical process temperature ofthe hot white liquor, polysulfide white liquor is not stable at all. This fact has disabled the use of polysulfide in the modern displacement kraft pulping processes developed for higher energy and chemical economy and improved pulp quality.

During the early 80's, new energy efficient kraft batch processes using various liquor displacements emerged. Characteristic for the displacement kraft batch process is to recover hot black liquor from the end of the cooking by displacement and then re-use the energy in the subsequent batches. Partly this is done by using the hot spent cooking liquor as such, and partly by heating the white liquor with the heat of the hot spent liquor leaving the digester system or collected for re-use at low temperature. This process arrangement leads to high temperatures in the input liquor accumulators. A low temperature white liquor, typically at 80 °C in the storage tank after re-causticization, cannot be used anymore, and the environment for stable polysulfide in the white liquor does not exist anymore.

Good examples of the development of displacement batch processes are given in, e.g., Fagerlund, U.S. Pat 4,578,149 and Östman, U.S. Pat 4,764,251. A further characteristic feature of a modern displacement batch process is to combine energy efficiency and efficient use of residual and fresh cooking chemicals to achieve, in addition to energy efficiency, high pulp strength and good delignification through hydroxyl and hydrosulfide concentration and temperature profiling at different stages of the cooking cycle (Hiljanen, Tikka, EP-B 520 452, Tikka, U.S. Pat 5,183,535).

EP 0 810 321 A1 discloses a batch process for the preparation of kraft pulp from lignin-containing cellulosic material, comprising the steps of adding to a vessel containing cellulosic material a volume of uncausticized cooking liquor, filling said vessel with spent cooking liquor, impregnating the cellulosic material with the resulting mixture of the uncausticized cooking liquor and spent cooking liquor, displacing the liquor used for impregnation with another volume of hot spent cooking liquor and pretreating the cellulosic material with said other volume of hot spent cooking liquor, displacing the liquor used for pretreatment with causticized hot cooking liquor and cooking the cellulosic material with said causticized hot cooking liquor to a desired degree of delignification, displacing the liquor used for cooking with wash filtrate, collecting a first volume of hot spent cooking liquor corresponding to the total volume required for pretreatment of the cellulosic material and of optional additions in other filling stages of a subsequent batch, and collecting a second volume of displaced liquor to be cooled and used in the impregnation of the cellulosic material in a subsequent batch.

Further, from WO 99/14423 a process for producing pulp from cellulosic fiber material with polysulfide regeneration in combination with polysulfide cooking is known. The cellulosic fiber material is impregnated with polysulfide before cooking followed by extraction of spent cooking liquor. A portion of the spent cooking liquor is gasified to hydrogen sulphide and treated to form an acidic gas comprising hydrogen sulphide and carbon dioxide. The acidic gas is reacted under conditions providing a hot stream of elemental sulphur, admixing thereby said stream with an alkaline liquor containing sulphide. In such a way an alkaline polysulfide liquor is formed which is added during cooking or impregnation, wherein during cooking a portion of the extracted spent cooking liquor is recycled to the impregnation step and a desired polysulfide concentration in the impregnation step is maintained by adding polysulfide liquor.

The strive for higher pulp yield is easy to understand. It is always more profitable to produce more pulp from a certain wood amount. The pulping industry has faced increasing environmental pressure to radically cut down environment polluting effluents. Reduction of the organic effluents from pulp bleaching requires kraft cooking to be extended to yield much lower residual lignin concentration in the pulp than before. Extended cooking means more carbohydrate losses. In order to enable extended cooking while improving energy economy and pulp quality, one popular option for the industry has been to use modern displacement batch cooking technology. In spite of all the advantages of this technology, it has not been possible to take the pulp yield advantage by using polysulfide white liquor. The present invention overcomes these problems and enables an efficient use of polysulfide by a novel displacement batch cooking process.

The use of anthraquinone (AQ) as a cooking catalyst is well known. It acts by reducing carbohydrate end groups, stabilising them against alkaline peeling and producing anthrahydroquinone, which is alkali soluble. Anthrahydroquinone reduces lignin, making it more reactive. In this process, anthraquinone is formed again and may react with carbohydrates.

During operation of displacement batch cooking processes, it has been observed that the properties of the black liquor originating from the early stages of the cook differ from those of black liquor from a traditional cook. Recycled black liquor originating from the early stages of the cooking sequence may complicate the evaporation of black liquor. A particular problem is fouling of the surfaces of heat exchangers in the evaporation plant, leading to a decrease in heat transfer. These evaporator fouling problems are typically related to calcium. In the early stage of alkaline cooking, calcium-containing material dissolves into the black liquor from the lignocellulosic material. In a traditional cook, the cook proceeds with heating, the temperature increases and no essential liquor exchange occurs. Then, a major part of the dissolved calcium-containing material in the cooking liquor is broken down, calcium carbonate is formed and as a result, a major part of the calcium is resorbed onto the lignocellulosic material in the digester. Following such a cooking process, evaporation of the black liquor can normally be carried out without problems caused by precipitation of calcium. In contrast, the evaporation problems with black liquors originating from the early stages of cooking are typically related to calcium-containing material dissolved in the early stages of a cook. The dissolved calcium-containing material has not been degraded, and the amount of calcium bound to the dissolved material in the black liquor is high. As disclosed in publication EP 1 242 674, this problem may be solved by re-introducing liquor having a high calcium precipitating potential into the digester as a displacement liquor at the end of a cook. At this point, the digester temperature is sufficiently high to cause calcium liberation. The calcium is then removed together with the pulp, and does not enter the evaporation and regeneration cycle.

### SUMMARY OF THE INVENTION

In accordance with the present invention, a method for producing pulp using polysulfide white liquor has been provided. The method involves a kraft batch process which comprises the addition of polysulfide white liquor in the impregnation and pretreatment in the very 'front end' of the cooking process, and a finalizing delignification stage with white liquor and optional cooking catalyst addition, which is facilitated by the modified 'front-end' process chemistry resulting in improved pulp yield. A volume of polysulfide white liquor is added as the first portion of liquor to enter the digester, or admixed with the impregnation liquor prior to this being pumped into the digester. For the purpose of this disclosure, "impregnation liquor" means a liquor stored at a temperature below its atmospheric boiling point, used for a first immersion of the lignocellulosic raw material in a batch pulping process.

In the present invention, lignocellulosic material entering a displacement batch process is thus pretreated with polysulfide- containing process liquors in conditions favourable for pre-treatment and polysulfide stability. A set of displacement batch process arrangements, capable of taking advantage of the polysulfide white liquor, are presented. The required dose of fresh polysulfide white liquor is introduced in the initial stage of the process. The impregnation stage provides for both impregnation and polysulfide pre-treatment reactions. An impregnation liquor circulation collects the displaced impregnation liquor which is re-used to fill and pressurize the digester after the first fresh liquor fill. As a result, the polysulfide concentration and dosage remain at a high level, and only the liquor balance excess is left over to be sent to chemicals recovery or re-use later in the cooking sequence. The displacement cooking process sequence then continues with hot fills of black and white liquors, cooking and final displacement.

An optional feature in the present invention is a new way to use a cooking catalyst, such as anthraquinone (AQ). As the generation of polysulfide white liquor decreases the concentration of hydrosulfide ions, the delignification rate is slower, reducing cooking capacity. The cooking catalyst can be used to maintain a normal kraft cooking rate and production level. In the present invention, the catalyst may be introduced into the digester together with the hot white liquor. By this means it will not escape due to displacements, and on the other hand, it arrives in the hot cooking stage where it is most needed. As a result, the technical and economical benefits of the displacement batch cooking are retained, while the advantages ofpolysulfide and cooking catalyst can be fully exploited.

### BRIEF DESCRIPTION OF THE FIGURES

Figure 1 shows a block diagram of a kraft displacement batch cooking system according to the invention. The top of the figure defines the required tanks, leaving or entering streams denoted by letters. The cooking stage sequence is displayed therebelow, chronologically starting from the top and the vertically indicated streams representing the liquors passing through the digester during the various stages. The letters denoting the various entering and leaving streams correspond to the source or destination in the tank scheme.
Figure 2 shows a further embodiment of a kraft displacement batch cooking system according to the invention.

### DISCLOSURE OF THE INVENTION

In the following, the method ofthe invention is disclosed in detail with reference to the attached Figure 1. It is understood, that liquor is charged from the digester bottom and displaced gases and liquor leave from the top.

The kraft batch cook is started by charging the digester with wood chips, or with another lignocellulosic material. After the lignocellulosic material charge, the digester is filled in a stepwise sequence using a volume of fresh polysulfide white liquor X1 from polysulfide white liquor tank 6, and impregnation liquor A1 from tank 4, topping the digester full of liquor. The volume of polysulfide white liquor may be added as a separate first portion, forming a raising pad of liquor as further liquor is pumped in from below. Alternatively, the polysulfide white liquor is mixed into the impregnation liquor.

An overflow, A2, conducted to the impregnation liquor tank 4, is preferred in order to remove air and the diluted first front of liquor. After the flow A2 is stopped, the digester is pressurized and impregnation is completed during an appropriate period of time. The cooking process is then continued by pumping in a volume of hot black liquor B1 from hot black liquor accumulator 1. The cooler impregnation liquor A3, displaced by hot black liquor, is conducted to impregnation liquor tank 4 to be re-used in subsequent batches. Pumping a volume C of hot white liquor from tank 3 into the digester then continues the cooking sequence. Together with white liquor C, an amount of cooking catalyst may be dosed into the digester. The liquor D1, displaced by hot liquor above about the atmospheric boiling point, in conducted to hot black liquor accumulator 2.

At the end of the sequence described above, the digester is close to the final cooking temperature. The final heating-up is carried out using direct or indirect steam heating and digester re-circulation. After the desired cooking time when the delignification has proceeded to the desired final reaction degree, the spent liquor is ready to be displaced with wash filtrate E1 from tank 5. A volume A4 from impregnation liquor tank 4 may be used as a first portion of displacement liquor in order to deactivate the potential scale-forming calcium therein, as disclosed in EP 1 242 674.

In the final displacement, the first displaced volume B2 displaced by wash filtrate is conducted to black liquor accumulator 1. The second portion D2 of displaced black liquor, which is diluted by the wash filtrate but is still above atmospheric boiling point, is conducted to the hot black liquor accumulator 2. After completed final displacement, the digester contents are discharged for further processing of the pulp. The above cooking sequence may then be repeated.

The hot black liquor from accumulator 2 is conducted to the evaporation plant, first being used to heat white liquor due for tank 3, and/or water, by means ofheat exchange.

Tank 6 is provided for storage of polysulfide white liquor, supplied from a plant for polysulfide generation.

### DESCRIPTION OF PREFERABLE EMBODIMENTS

In the following, reference is made to the figure described in the preceding section.

In the process of the present invention, a volume of polysulfide white liquor, corresponding to 25-90 % of the total active alkali dosage and resulting in 0,5% to 5% polysulfide dosage on abs, dry wood is added into the digester before the impregnation fill is completed. Impregnation is carried out using temperature of between 70 °C and 120 °C, preferably between 85 - 95 °C, and a time of between about 20 to about 120 minutes, preferably between about 30 to about 60 minutes, more preferably between about 25 to about 40 minutes.

In a preferable embodiment, the polysulfide white liquor is added as a separate portion before the introduction of further liquor.

In a preferable embodiment, the volume ofpolysulfide white liquor corresponds to 50-75 % of the total active alkali dosage for the relevant batch.

In accordance with a particular embodiment of the process of the present invention, a cooking catalyst is used. Preferable catalysts are anthraquinone, anthraquinone sulfonate, and hydroanthraquinone. Any other appropriate redox-catalyst as anticipated by those skilled in the art may be used.

In accordance with an alternative embodiment of the process of the present invention, the following fractions displaced from the digester:
- hot cooking spent liquor fraction B2 and
- fractions D1 and D2, which are of lower temperature and poorer in chemicals, are collected in a single accumulator to be used in the hot black liquor pretreatment stage. In this configuration, hot black liquor accumulators 1 and 2 of Figure 1 are combined. The black liquor flow to the evaporation plant is drawn from the single hot black liquor accumulator, the stream being used to heat, by means of heat exchange, white liquor heading for white liquor accumulator 3, and/or water, as shown for tank 2 in Fig 1.

If high dosages ofpolysulfide white liquor are used in the impregnation stage ofthe process, longer impregnation times than in the prior art and/or a two accumulator system and/or impregnation liquor transfer to hot black liquor tank 1 may be used in order to avoid too high a residual alkali concentration in the feed of the evaporation plant. Thus, in accordance with a further embodiment of the process of the present invention, shown in Figure 2, a volume of impregnation liquor from impregnation tank 4 is conducted to hot black liquor tank 1 to be used in hot black liquor treatment, B 1. The stream from impregnation liquor tank 4 to hot black liquor tank 1 may be heated by means of heat exchange with the stream from hot black liquor accumulator 2 to the evaporation plant.

In addition to the white liquor charge prior to the cooking stage, one or more additional white liquor charges may be carried out during the cook.

The principal advantage of the process of the present invention is that the `front-end' of the kraft displacement batch cooking system is rendered more effective from a chemical point of view, and in regard to process arrangements. The polysulfide charge used reflects the improvement in pulp yield from the digested lignocellulosic material.

The following examples are illustrative of the invention. The following abbreviations are used:
- WBL: Warm impregnation black liquor
- DWBL: Displaced WBL (from the digester)
- HBL: Hot black liquor
- RHBL: Displaced HBL (from the digester)
- DCBL: Displaced cooking black liquor
- WF: Wash filtrate
- PSWL: Polysulfide white liquor

### Production of a normal `reference' pine kraft pulp using the displacement kraft batch technique:

4,0 kg pine (*Pinus sylvestris*) chips (oven dry basis) were metered into a chip basket positioned in a 20-litre jacketed displacement batch digester. The lid of the digester was closed. Impregnation black liquor, consisting of wash filtrate and white liquor (WBL, 80-90°C, 25 gEA/1) was pumped in during app. 10 minutes followed by impregnation at 90°C under 2,5 bar overpressure. The duration of the impregnation stage was 40 minutes (WBL-fill and impregnation in total). After impregnation, a hot black liquor pre-treatment stage was commenced by introducing hot black liquor (HBL 1, 150°C, app. 20 gEA/1) to the bottom of the digester, displacing the spent impregnation liquor (DWBL) out from the top of the digester. The hot black liquor pre-treatment stage duration was 30 minutes. After hot black liquor pre-treatment stage, hot white liquor (121 gEA (NaOH)/1, sulfidity 37%) charge was introduced into the digester bottom displacing the corresponding volume of spent hot black liquor (RHBL) out of the digester. A 45 minute heat-up sequence with cooking liquor circulation raised the temperature from 150°C to the cooking temperature of 167°C. At 250 H-factors, a white liquor charge was introduced into the digester bottom displacing the corresponding volume of spent hot black liquor out of the digester (DCBL 1). After the cooking time fulfilled the target H-factor, terminal displacement was started by introducing cool DWBL and wash filtrate (WF) in a sequence into the digester bottom displacing the hot spent black liquor out of the digester top (DCBL 2). The first displaced portion the hot black liquor with the hot black liquor displaced earlier during the cooking sequence (DCBL 2 + DCBL 1) covered the volume needed for the next cook's hot black liquor (HBL 1). The terminal displacement stage duration was approximately 40 minutes. After the terminal displacement, the pulp was disintegrated, washed with deionised water, screened and analysed. The cooking procedure was repeated and thus equilibrium in the cooking process was obtained and the cooks started to repeat themselves corresponding to the industrial batch cooking system.

The experimental set-up to produce pulp according to the invention is described below.

4,0 kg pine (*Pinus sylvestris*) chips (oven dry basis) were metered into a chip basket positioned in a 20-litre jacketed displacement batch digester. The lid of the digester was closed. The chips were steamed until the digester temperature was 100°C, approximately 5 minutes. Impregnation liquors were introduced as sequence as follows: initially polysulfide white liquor black liquor (PSWL, volume according to the charge, app. 4,5-51); subsequently re-circulated spent impregnation liquor (DWBL) to hydraulically fill the digester. The impregnation fill sequence took app. 11-13 minutes and was followed by impregnation at 90°C under 2,5 bar overpressure. The duration of the impregnation stage was 40 minutes (fill sequence and impregnation in total). After impregnation, a hot black liquor pre-treatment stage was carried out by introducing hot black liquor (HBL 1, 150°C, app. 20 gEA/1) to the bottom of the digester of the digester, displacing the spent impregnation liquor from the top of the digester (DWBL). The hot black liquor pretreatment stage duration was 30 minutes. After the hot black liquor pre-treatment stage, hot white liquor (121 gEA (NaOH)/1, sulfidity 37%) charge was introduced, displacing the corresponding volume of spent hot black liquor from the digester (RHBL). Together with the WL, a cooking catalyst was charged mixed with a small volume of hot black liquor. A 45 minute heat-up sequence with cooking liquor circulation raised the temperature from 150°C to the cooking temperature of 167 °C. At 250 H-factors, a further white liquor charge was introduced into the digester bottom displacing the corresponding volume of spent hot black liquor from the digester (DCBL 1). After the cooking time fulfilled the target H-factor, terminal displacement was started by introducing a volume of cool DWBL and wash filtrate (WF) in a sequence into the digester bottom displacing the hot spent black liquor out of the digester top (DCBL 2). The first displaced portion of hot black liquor together with the hot black liquor displaced earlier during the cooking sequence (DCBL 2 + DCBL 1) covered the 171 volume needed for the next cook's hot black liquor (HBL 1). After the terminal displacement, the pulp was disintegrated, washed with deionised water, screened and analysed. The cooking procedure was repeated, equilibrium in the cooking process was reached and the cooks started to repeat themselves corresponding to the industrial batch cooking system.

### Example 1. Demonstration of yield improvement using polysulfide white liquor addition

The reference cook follows the same addition and temperature sequences as the cooks according to the invention. All cooks were digested to the same target kappa number. A clear yield improvement correlating with polysulfide addition can be observed

| Cooking model | PS-charge, % on wood | Kappa number | Total yield, % on wood | Rejects, % on wood |
|---|---|---|---|---|
| Reference | Nil | 25,9 | 44,0 | 0,26 |
| SB-PSAQ | 1,21 | 25,9 | 45,8 | 0,36 |
| SB-PSAQ | 1,58 | 25,8 | 46,8 | 0,24 |

### Example 2. The effect of anthraquinone to preserve the rate of delignification during cooking

It is seen, that the reference cook requires a significantly higher H-factor to reach the target kappa number.

| Method | PSWL in imp, % | PS, % on wood | H-factor | EoC, g/l | Kappa# | Yield, % on wood | Reject, % on wood |
|---|---|---|---|---|---|---|---|
| Reference | - | - | 1285 | 16 | 26,9 | 43,6 | 1,01 |
| PS pad, AQ 0% | 70 % | 1,45 | 1106 | 19,1 | 27,1 | 44,3 | 0,15 |
| PS pad, AQ 0,05% | 70 % | 1,45 | 1030 | 19,9 | 26,7 | 44,5 | 0,16 |
| PS pad, AQ 0,1% | 70 % | 1,45 | 1096 | 18,1 | 27,3 | 45,8 | 0,1 |

## Claims

1. A batch process for the preparation of kraft pulp with improved yield from lignin-containing cellulosic material, comprising the steps of
- filling and pressurizing a digester containing the cellulosic material with impregnation liquor collected from a previous batch, said impregnation liquor admixed with, or preceded by an addition of, a volume of polysulfide white liquor,
- impregnating the cellulosic material with the resulting mixture of impregnation liquor,
- displacing the impregnation liquor with hot spent cooking liquor,
- reacting the impregnated cellulosic material with said hot spent liquor,
- displacing hot spent cooking liquor with a volume of hot white liquor and cooking the cellulosic material with said white liquor to a desired degree of delignification, and
- displacing the liquor used for cooking.

2. The process of claim 1, wherein the amount of polysulfide white liquor added corresponds to 25-90 % of the total active alkali dosage for the batch.

3. The process of claim 1, wherein the amount of polysulfide white liquor added corresponds to 50-75 % of the total active alkali dosage for the batch.

4. The process of claim 1, wherein the polysulfide dosage corresponds to 0,5-5 % relative to abs, dry wood.

5. The process of claim 1, wherein the volume of polysulfide white liquor is added separately to the digester before the impregnation liquor.

6. The process of claim 1, wherein an amount of cooking catalyst is added to the hot white liquor.

7. The process of claim 6, wherein the cooking catalyst is anthraquinone, anthraquinone sulfonate, hydroantraquinone or a redox-catalyst derivative thereof.

8. The process of claim 1, wherein hot spent liquor displaced from the digester is collected in a single hot liquor tank.

9. The process of claim 1, wherein after the cooking is finished, a volume of impregnation liquor is introduced into the digester as the first volume of displacement liquor.

10. The process of claim 1, wherein a volume of impregnation liquor is transferred from an impregnation liquor tank to a hot spent cooking liquor tank.

11. The process of claim 10, wherein the digester system comprises two hot spent liquor tanks.

## Patentansprüche

1. Batch-Prozess für die Herstellung von Kraftzellstoff mit verbesserter Ausbeute aus Lignin enthaltendem Cellulosematerial mit den Schritten
- Befüllen und Unter-Druck-Setzen eines das Cellulosematerial enthaltenden Digestors zusammen mit einer aus einem vorherigen Batch gesammelten Imprägnierungslauge, wobei die Imprägnierungslauge einem Volumen Polysulfid-Weisslauge zugemischt wird oder ein Hinzufügen von diesem vorangegangen ist,
- Imprägnieren des Cellulosematerials mit dem erhaltenen Gemisch aus Imprägnierungslauge,
- Verdrängen der Imprägnierungslauge mit heißer Kochablauge,
- Umsetzen des imprägnierten Zellulosematerials mit der heißen Ablauge,
- Verdrängen der heißen Kochablauge mit einem Volumen heißer Weisslauge und Kochen des Zellulosematerials mit der Weisslauge bis zu einem gewünschten Ligninentfernungsgrad und
- Verdrängen der zum Kochen verwendeten Lauge.

2. Prozess nach Anspruch 1, bei dem die hinzugefügte Menge an Polysulfid-Weisslauge 25 - 90 % der gesamten aktiven Alkalidosis für das Batch entspricht.

3. Prozess nach Anspruch 1, bei dem die hinzugefügte Menge an Polysulfid-Weisslauge 50 - 75 % der gesamten aktiven Alkalidosis für das Batch entspricht.

4. Prozess nach Anspruch 1, bei dem die Polysulfiddosis 0,5 - 5 % relativ zu abs. trockenem Holz entspricht.

5. Prozess nach Anspruch 1, bei dem das Volumen an Polysulfid-Weisslauge dem Digestor separat vor der Imprägnierungslauge zugefügt wird.

6. Prozess nach Anspruch 1, bei dem der heißen Weisslauge eine Menge an Kochkatalysator hinzugefügt wird.

7. Prozess nach Anspruch 6, bei dem der Kochkatalysator Anthraquinon, Anthraquinonsulfat, Hydroanthraquinon oder ein Redoxkatalysator-Derivat davon ist.

8. Prozess nach Anspruch 1, bei dem aus dem Digestor verdrängte heiße Ablauge in einem einzelnen Heißlaugetank gesammelt wird.

9. Prozess nach Anspruch 1, bei dem nach Beendigung des Kochens ein Volumen an Imprägnierungslauge als das erste Volumen an Verdrängungslauge in den Digestor eingeführt wird.

10. Prozess nach Anspruch 1, bei dem ein Volumen an Imprägnierungslauge von einem Imprägnierungslaugetank zu einem Tank mit heißer Kochablauge transportiert wird.

11. Prozess nach Anspruch 10, bei dem das Digestorsystem zwei Tanks mit heißer Ablauge umfasst.

## Revendications

1. Procédé discontinu pour la préparation de pâte kraft ayant un rendement amélioré à partir d'une matière cellulosique contenant de la lignine, comprenant les étapes de
- remplissage et mise sous pression d'un lessiveur contenant la matière cellulosique avec une liqueur d'imprégnation récupérée d'un lot précédent, ladite liqueur d'imprégnation mélangée avec, ou précédée de l'addition, d'un volume de liqueur blanche de polysulfure,
- imprégnation de la matière cellulosique avec le mélange résultant de liqueur d'imprégnation,
- déplacement de la liqueur d'imprégnation avec de la liqueur de cuisson usée chaude,
- réaction de la matière cellulosique imprégnée avec ladite liqueur usée chaude,
- déplacement de la liqueur de cuisson usée chaude avec un volume de liqueur blanche chaude et cuisson de la matière cellulosique avec ladite liqueur blanche jusqu'à un degré désiré de délignification, et
- déplacement de la liqueur utilisée pour la cuisson.

2. Procédé selon la revendication 1, dans lequel la quantité de liqueur blanche de polysulfure ajoutée correspond à 25-90% de la dose alcaline active totale pour le lot.

3. Procédé selon la revendication 1, dans lequel la quantité de liqueur blanche de polysulfure ajoutée correspond à 50-75% de la dose alcaline active totale pour le lot.

4. Procédé selon la revendication 1, dans lequel la dose de polysulfure correspond à 0,5-5% par rapport au bois sec absolu.

5. Procédé selon la revendication 1, dans lequel le volume de liqueur blanche de polysulfure est ajouté séparément dans le lessiveur avant la liqueur d'imprégnation.

6. Procédé selon la revendication 1, dans lequel une quantité de catalyseur de cuisson est ajoutée à la liqueur blanche chaude.

7. Procédé selon la revendication 6, dans lequel le catalyseur de cuisson est de l'anthraquinone, du sulfonate d'anthraquinone, de l'hydroanthraquinone ou un dérivé catalyseur d'oxydoréduction de ceux-ci.

8. Procédé selon la revendication 1, dans lequel la liqueur usée chaude déplacée du lessiveur est récupérée dans un réservoir unique de liqueur chaude.

9. Procédé selon la revendication 1, dans lequel, lorsque la cuisson est terminée, un volume de liqueur d'imprégnation est introduit dans le lessiveur en tant que premier volume de liqueur de déplacement.

10. Procédé selon la revendication 1, dans lequel un volume de liqueur d'imprégnation est transféré d'un réservoir de liqueur d'imprégnation dans un réservoir de liqueur de cuisson usée chaude.

11. Procédé selon la revendication 10, dans lequel le système de lessiveur comprend deux réservoirs de liqueur usée chaude.
